

[54] SILVER BROMOIODIDE PHOTOGRAPHIC EMULSION WITH IMPROVED GREEN SENSITIVITY

[75] Inventors: Hirozo Ueda; Keisuke Shiba; Akira Sato, all of Kanagawa, Japan

[73] Assignee: Fuji Photo Film Co., Ltd., Minami Ashigara-shi, Kanagawa, Japan

[22] Filed: Oct. 30, 1972

[21] Appl. No.: 301,912

[30] Foreign Application Priority Data

Oct. 28, 1971 Japan..... 46-85835

[52] U.S. Cl..... 96/124, 96/108, 96/125,  
96/137

[51] Int. Cl..... G03c 1/14, G03c 1/18

[58] Field of Search ..... 96/137, 124, 108, 125

[56] References Cited

UNITED STATES PATENTS

3,178,292 4/1965 Fix ..... 96/108

|           |        |                     |         |
|-----------|--------|---------------------|---------|
| 3,436,221 | 4/1969 | Sprung.....         | 96/108  |
| 3,457,072 | 7/1969 | Ditzer et al. ....  | 96/94 R |
| 3,531,288 | 9/1970 | Jones .....         | 96/108  |
| 3,594,172 | 7/1971 | Sincius.....        | 96/108  |
| 3,745,015 | 7/1973 | Van Pee et al. .... | 96/108  |

Primary Examiner—J. Travis Brown

Attorney, Agent, or Firm—Sughrue, Rothwell, Mion,  
Zinn & Macpeak

[57] ABSTRACT

In a silver bromoiodide photographic emulsion containing at least one green sensitizing dye, a silver bromoiodide photographic emulsion wherein at least 0.01 mol percent of iodide ion based on silver halide adsorbs on the surface of silver bromoiodide grains contained in the emulsion.

32 Claims, No Drawings

**SILVER BROMOIODIDE PHOTOGRAPHIC  
EMULSION WITH IMPROVED GREEN  
SENSITIVITY**

**BACKGROUND OF THE INVENTION**

**1. Field of the Invention**

The present invention relates to a silver bromoiodide emulsion comprising crystalline grains containing mixed crystals of silver bromoiodide having iodide ions and one or more sensitizing dyes absorbed on the surface thereof and, more particularly, it relates to an improved silver bromoiodide photographic emulsion suitable for spectral sensitization to green light.

**2. Description of the Prior Art**

In the photographic emulsion-producing art, it has heretofore been well known that the spectral sensitivity of a photographic emulsion can be extended from the spectral sensitivity intrinsic to the silver halide (mainly ranging from the near ultraviolet region to the blue light region) to visible light of longer wavelengths or to the infrared region by the addition of dyes of the cyanine series to the photographic emulsion. This procedure is termed spectral sensitization.

The above-described procedure has enabled the art to markedly increase the usefulness of photographic materials utilizing silver halides as a light-sensitive element. Especially from the viewpoint of practical usage, spectral sensitization gives the silver halide a good parallelism with the spectral response of human eyes, and this produces a good reproduction of natural colors with a silver halide system. Moreover, the development of scientific uses such as infrared detectors and the like were also made possible.

A variety of combinations of dyes and photographic emulsions have been developed in order to use the above-mentioned spectral sensitization, depending on the purpose of the particular photographic light-sensitive material. The dye/emulsion combination is the main factor that determines in which spectral region the emulsion is sensitized, and how much sensitivity the emulsion is provided. Furthermore, a number of inventions have been made to improve the emulsions with respect to other desirable characteristics such as rapid processing capability, good storage capability of the light-sensitive material and latent images thereon, lowered color stain in the processed light-sensitive materials and the like, by the use of a specific dye/emulsion combination.

However, in spite of extensive investigation no completely satisfactory dye/emulsion combination has been proposed which satisfies all of the above factors for a specific emulsion.

For example, in the case of recording a green object, a difficulty arises from the fact that the main spectral reflection region of the green of the leaves of natural plants usually lies at about 550 nm, while the main spectral reflection region of artificial green (such as the green of artificial plants, e.g., Hong-Kong flowers, and that of different types of printed material) lies in the range of from 510 to 530 nm. In practice, it is not always easy to provide a photographic emulsion with a spectral sensitivity capable of obtaining a good reproduction of both greens at the same time.

In addition, in the case of designing a light-sensitive material for color prints, it is often necessary to adjust the spectral sensitivity or the light-sensitivity of the

light-sensitive material for duplication or printing within a range of from about 5 to about 10 nm, according to the spectral absorption region of the dyes used in the original color photographic image. However, this is not necessarily a simple matter either, as when the spectral absorption region is shifted to a desired region by slight modification of the chemical structure of the spectrally sensitizing dyes in order to shift the spectral sensitivity by only about 5-20 nm, accompanying difficulties often occur, e.g., the sensitivity is greatly changed, the rate of development is changed, the storage property is affected, color stain left on the processed material is visually increased, etc.

**SUMMARY OF THE INVENTION**

Therefore, the object of the present invention is to provide a silver halide photographic emulsion capable of markedly improving the above-described difficulties, more specifically, an object of the present invention is to provide a photographic emulsion in a gelatino-silver bromoiodide photographic light-sensitive material wherein spectral sensitization in the green region is provided in a desired spectral wavelength region without encountering the above-described secondary defects.

The present inventors have found that in the case of the spectral sensitization of a silver bromoiodide photographic emulsion to the green region substantially constant high green sensitivity can be obtained, even when a series of green light absorbing and spectral sensitizing dyes whose spectral absorption regions are a little different from each other are used, by adsorbing iodide ions onto the silver bromoiodide grains and adjusting the amount of the iodide ion adsorbed according to the kind of spectral sensitizing agents used.

**DETAILED DESCRIPTION OF THE INVENTION**

It could not have been expected from the prior art that the spectral sensitivity region could be precisely adjusted as desired without encountering the aforesaid difficulties, i.e., changes in sensitivity, etc., as described above.

It is a remarkable technical progress that the present invention makes it extremely easy to design a light-sensitive material according to the desired end use of the element.

In a silver bromoiodide emulsion, iodide ions are, of course, included in the grains as a mixed crystal, and hence it would naturally be supposed that a certain amount of iodide ions exist on the surface of the grains. It is therefore a surprising discovery that, in spite of the above fact, a certain addition amount of iodide ions provides marked effects from the viewpoint of spectral sensitization.

In general, it has been known that iodide ions can sometimes be added accidentally to a photographic emulsion together with spectral sensitizing dyes. That is, many of the cyanine dyes frequently employed as spectral sensitizing dyes are cationic dyes, and when these dyes have an iodide ion as a counter ion, iodide ions are added to the photographic emulsion together with the dye cations without any intention of doing such, and they sometimes adsorb on the silver halide grains. However, the molar amount of iodide ions added in such a situation is equal to that of the dye(s) added (That is, conventionally, this amount is very small, as compared with that of the present invention.).

so that the effect obtained by adjusting the iodide ion amount added as described in the present invention is not shown.

The spectral sensitizing dyes used in the present invention are known, for example, they are described in Japanese Pat. publication No. 22884/68, West German Pat. OLS No. 2,030,326, etc.

It is described in Japanese Pat. publication No. 22884/68 that spectral sensitivity can be changed by altering the characteristics of the emulsion, above all, by a change in the silver ion concentration. It is true that the adsorption of iodide ions will naturally cause some change in the silver ion concentration, but the effect of the adsorbed iodide ions in a silver bromoiodide system could not be expected from prior art as described above. In addition, the present invention tends in the direction of reducing the silver ion concentration, which is quite opposite to the direction of "increasing the silver ion concentration to raise the spectral sensitivity" as is described in the known literature cited above.

The procedure of preparing the photographic emulsion of the present invention having high green sensitivity will be more specifically described below.

The silver halide photographic emulsion contains silver bromoiodide mixed crystals preferably containing about 0.5 to about 10 mol percent of iodide ions and, as a protective hydrophilic colloid, a major proportion of gelatin. Other protective colloid conventionally used in the art, such as phthalated gelatin, polyacrylic amide, polyvinylalcohol, polyvinylpyrrolidone, may be used, of course. Generally the ratio of silver iodobromide to protective colloid is from about 3:1 to about 1:3, by weight. This is not overly critical, however, and greater and lesser proportions can be used.

The mean grain size of the silver bromoiodide usually ranges from 0.2 to 2 - 3  $\mu$  in diameter, of course, finer or larger grain size silver halide may be used in the present invention. (refer, for example, to Trivelli Smith "Empirical relations between sensitometric size frequency characterized in photographic series, Photographic Journal" vol LXXIX page 330 - 338(1939)) These grains are usually subjected to various sensitizing processes usually known as chemical ripening (such as sulfur sensitization, noble metal sensitization, reduction sensitization and the like).

The iodide ions are usually added to the system as a water-soluble iodide ion compound, generally added to the silver bromoiodide photographic emulsion sol in the form of an aqueous solution. The water-soluble iodide ion compound is preferred to be completely soluble or substantially soluble in water. The term "water-soluble" implies at least 10 weight percent solubility as a practical matter. As the water-soluble iodide ion compounds, there can be illustrated salts, for example, alkali metal salts such as sodium iodide and potassium iodide;  $CoI_2$ ; amine salts such as ammonium iodide; and alkali earth metal such as  $ZnI_2$ ,  $CdI_2$ ,  $CaI_2$ ,  $SrI_2$  and  $BaI_2$ . The proportion of iodide ions added, based on the silver bromoiodide, is at least 0.01 mol percent and preferably no more than 1.0 mol percent, most preferably 0.05 to 0.3 mol percent, which is suitably adjusted depending upon the kind of the sensitizing dye and emulsion.

Alternatively, an iodide ion compound and a bromide ion compound (the molar ratio  $Br/I^-$  is operable in a range of from 1 to 30) may be mixed to form an

aqueous solution, and added to a sol-state silver bromoiodide emulsion. This concentration of iodide and/or bromide is in addition to any bromide or iodide present throughout the grains as mixed silver halide. This procedure may give more reproducible results with the invention than the single addition of iodide.

The aqueous solution containing iodide ions is added to the emulsion and sufficiently stirred. Substantially all of the iodide ions added are believed to immediately absorb on the silver bromoiodide grains. This is easily recognized by an immediate change in color of the grains.

To the resulting silver bromoiodide photographic emulsion (maintained in the sol state) to which iodide ions have been added there is added an organic solution of a spectral sensitizing dye which provides green sensitivity. Generally from about  $10^{-4}$  to about  $2 \times 10^{-2}$  moles of green sensitizing dye (or dyes) is added per mole of silver halide. Use of a substantially lesser amount may provide lessened effects, whereas no overly significant increase is encountered by using substantially greater amounts.

The term "green sensitizing dye" includes both an anionic dye and a cationic dye with or without an iodide ion as a counter anion.

As the green sensitizing dye used in the present invention, cyanine dyes comprising an oxacarbocyanine skeleton, such as benzoxacarbocyanine, naphthoxacarbocyanine, etc. [group I], cyanine dyes comprising a benzimidazolocarbocyanine skeleton, a benzimidazoloxacarbocyanine skeleton or a benzimidazoloindocarbocyanine skeleton, such as benzimidazonaphthoxacarbocyanine, etc. [group II], are preferably used, either independently or in combinations of at least two dyes wherein one belongs to group I and one belongs to group II, or at least two dyes belonging to group II may be used. As used herein and in the appended claims, the term "cyanine" includes cyanine dyes and merocyanine dyes, e.g., monomethine cyanine dyes and carbocyanine dyes. As is well known from the article by Mees and James ("The Theory of Photographic Process," IIEd, 1966, pp. 201 - 202), cyanine dyes feature the amidinium ion chromophore system wherein each nitrogen atom is contained in a heterocyclic ring.

Illustrating the above in even more detail, preferably dyes represented by the following general formula (I) are used among the dyes belonging to group (I):



60 wherein  $A_1$  and  $A_3$  each represents a hydrogen atom or halogen atom (e.g., chlorine, bromine, iodine and fluorine),  $A_2$  and  $A_4$  represents a hydrogen atom, halogen atom, hydroxy group, alkoxy group (e.g., methoxy, ethoxy group, etc.), amino group (e.g., amino, methylamino, dimethylamino group, etc.), acylamido group (e.g., acetamido, propionamido group, etc.), acyloxy group (e.g., acetoxy group, etc.), alkoxy carbonyl group (e.g., methoxycarbonyl, ethoxycarbonyl, propoxycarbonyl group, butoxycarbonyl, etc.), lower alkyl group (e.g., methyl, ethyl, isopropyl group, etc.).

or alkoxycarbonylamino group (e.g., ethoxycarbonylamino group, etc.), or, when taken together,  $A_1$  and  $A_2$ , and  $A_3$  and  $A_4$ , can be the atoms necessary to form a benzene nucleus (in this case, the heterocyclic nucleus results in, for example, an  $\alpha$ -naphthoxazole nucleus,  $\beta, \beta'$ -naphthoxazole nucleus, or  $\beta$ -naphthoxazole nucleus),  $R$  represents a hydrogen atom, lower alkyl group (e.g., methyl, ethyl, n-propyl group, etc.), aryl group (e.g., phenyl, tolyl group, etc.) etc.  $R_1$  and  $R_2$  each represents an alkyl group (such as methyl, ethyl, n-propyl group), hydroxyalkyl group (e.g., 2-hydroxyethyl, 3-hydroxypropyl, 4-hydroxybutyl group, etc.), acetoxyalkyl group (e.g., 2-acetoxyethyl, 3-acetoxypropyl, 4-acetoxybutyl group, etc.), alkoxyalkyl group (e.g., 2-methoxyethyl, 3-methoxypropyl group, etc.), alkyl group containing a carboxyl group (e.g., carboxymethyl, 2-carboxyethyl, 3-carboxypropyl, 4-carboxybutyl, 2-(2-carboxyethoxy)ethyl group, etc.), an alkyl group containing a sulfo group (e.g., 2-sulfoethyl, 3-sulfopropyl, 4-sulfobutyl, 2-hydroxy-3-sulfopropyl, 2-(3-sulfopropoxy)ethyl, 2-acetoxy-3-sulfopropyl, 3-methoxy-2-(3-sulfopropoxy)propyl, 2-[2-(3-sulfopropoxy)-ethoxy]ethyl, p-sulfonylbenzyl, p-sulfophenethyl group, etc.), benzyl group, phenethyl group, vinyl-methyl group, and the like,  $X^-$  represents an acid anion (e.g., chloride, bromine, iodide, thiocyanate, methylsulfate, ethyl-sulfate, perchlorate, p-toluenesulfonate ion, etc.), and  $n$  represents 1 or 2. In the above formula,  $A_1$ ,  $A_2$ ,  $A_3$ ,  $A_4$ ,  $R$ ,  $R_1$  and  $R_2$  may be the same or different from each other.

Of the dyes belonging to group (II), those represented by the following general formula (2) are preferably used:



wherein  $B_1$  represents a hydrogen atom or halogen atom (e.g., chlorine, bromine, iodine, fluorine),  $B_2$ ,  $B_3$  and  $B_4$  each represents a hydrogen atom, halogen atom, lower alkyl group (e.g., methyl, ethyl, trifluoromethyl group, etc.), amino group (e.g., amino, methylamino, dimethylamino group, etc.), acylamido group (e.g., acetamido, propionamido group, etc.), acyloxy group

| Dye No. | B <sub>1</sub> | B <sub>2</sub> | B <sub>3</sub> | B <sub>4</sub>        | R <sub>3</sub>                | R <sub>4</sub>                                                | R <sub>5</sub>                                     | R <sub>6</sub> | Y                                | X     | m |
|---------|----------------|----------------|----------------|-----------------------|-------------------------------|---------------------------------------------------------------|----------------------------------------------------|----------------|----------------------------------|-------|---|
| 8       | 6-Cl           | 5-Cl           | II             | 5'-COOCH <sub>3</sub> | C <sub>2</sub> H <sub>5</sub> | (CH <sub>2</sub> ) <sub>3</sub> SO <sub>3</sub> <sup>-</sup>  | (CH <sub>2</sub> ) <sub>3</sub> SO <sub>3</sub> H  | II             | -O-                              | ----- | 1 |
| 9       | 6-Cl           | 5-Cl           | II             | 5'-Cl                 | C <sub>2</sub> H <sub>5</sub> | (CH <sub>2</sub> ) <sub>3</sub> SO <sub>3</sub> <sup>-</sup>  | (CH <sub>2</sub> ) <sub>3</sub> SO <sub>3</sub> H  | II             | -O-                              | ----- | 1 |
| 10      | 6-Cl           | 5-Cl           | II             | 5'-OCH <sub>3</sub>   | C <sub>2</sub> H <sub>5</sub> | (CH <sub>2</sub> ) <sub>3</sub> SO <sub>3</sub> <sup>-</sup>  | (CH <sub>2</sub> ) <sub>3</sub> SO <sub>3</sub> H  | II             | -O-                              | ----- | 1 |
| 11      | 6-Cl           | 5-Cl           | II             | 5'-CH <sub>3</sub>    | C <sub>2</sub> H <sub>5</sub> | (CH <sub>2</sub> ) <sub>3</sub> SO <sub>3</sub> <sup>-</sup>  | (CH <sub>2</sub> ) <sub>3</sub> SO <sub>3</sub> H  | II             | -O-                              | ----- | 1 |
| 12      | 6-Cl           | 5-Cl           | II             |                       | C <sub>2</sub> H <sub>5</sub> | (CH <sub>2</sub> ) <sub>3</sub> SO <sub>3</sub> <sup>-</sup>  | (CH <sub>2</sub> ) <sub>3</sub> SO <sub>3</sub> H  | II             | -O-                              | ----- | 1 |
|         |                |                |                |                       |                               |                                                               |                                                    |                |                                  |       |   |
| 13      | 6-Cl           | 5-Cl           | 6'-Cl          | 5'-Cl                 | C <sub>2</sub> H <sub>5</sub> | (CH <sub>2</sub> ) <sub>3</sub> SO <sub>3</sub> <sup>-</sup>  | (CH <sub>2</sub> ) <sub>3</sub> SO <sub>3</sub> H  | II             | >N-C <sub>2</sub> H <sub>5</sub> | ----- | 1 |
| 14      | 6-Cl           | 5-Cl           | 6'-Cl          | 5'-Cl                 | C <sub>2</sub> H <sub>5</sub> | (C <sub>2</sub> H <sub>5</sub> ) <sub>2</sub> O <sup>2-</sup> | (C <sub>2</sub> H <sub>5</sub> ) <sub>2</sub> O    | II             | >N-C <sub>2</sub> H <sub>5</sub> | ----- | 1 |
|         |                |                |                |                       |                               | (CH <sub>2</sub> ) <sub>3</sub> SO <sub>3</sub> <sup>-</sup>  | (CH <sub>2</sub> ) <sub>3</sub> SO <sub>3</sub> Na | II             |                                  |       |   |

(e.g., acetoxy group, etc.), alkoxycarbonyl group (e.g., methoxycarbonyl, ethoxycarbonyl, propoxycarbonyl, butoxycarbonyl group, etc.), carboxyl group, alkoxy group (e.g., methoxy, ethoxy group, etc.), aryl group (e.g., phenyl, tolyl group, etc.), cyano group, carbamoyl group (carbamoyl, methylcarbamoyl, phenylcarbamoyl, dimethylcarbamoyl, diethylcarbamoyl, morpholinocarbamoyl, piperidinocarbamoyl group, etc.), alkylsulfonyl group (e.g., methylsulfonyl group, etc.), alkylaminosulfonyl group (e.g., methylaminosulfonyl, ethylaminosulfonyl, dimethylaminosulfonyl, morpholinosulfonyl, piperidinosulfonyl, pyrrolidinosulfonyl group, etc.) or aminosulfonyl group, or, when taken together,  $B_3$  and  $B_4$  can represent the atoms necessary to form a benzene ring,  $Y$  represents  $-\text{O}-$ ,



20 wherein  $R_7$  and  $R_8$  each represents an alkyl group (e.g., methyl, ethyl, vinylmethyl group, etc.).



25 wherein  $R_6$  represents an alkyl group (such as a methyl-  
ethyl group),  $R_3$ ,  $R_4$  and  $R_5$  represent the same alkyl  
groups as  $R_1$  or  $R_2$ ;  $R_6$  represents a hydrogen atom or  
 $R_5$  and  $R_6$  may combine with each other through an al-  
30 kylene group (e.g., dimethylene, trimethylene group,  
etc.) ( $R_5$  often represents an alkylene group in the ben-  
zimidazoloindocarbocyanine dyes), and  $m$  represents 1  
or 2. In the above general formula (2),  $B_1$ ,  $B_2$ ,  $B_3$ ,  $B_4$ ,  
 $R_3$ ,  $R_4$ ,  $R_5$  and  $R_6$  may be the same or different from  
35 each other.

Specific examples of dyes used in the present invention are illustrated hereinafter, which in no way should be taken to limit the invention.

40 Examples of dyes belonging to those represented by general formula (1) are:

| Dye No. | A <sub>1</sub> | A <sub>2</sub>                                                                      | A <sub>3</sub> | A <sub>4</sub>                   | R                             | R <sub>1</sub>                                               | R <sub>2</sub>                                      | X | n |
|---------|----------------|-------------------------------------------------------------------------------------|----------------|----------------------------------|-------------------------------|--------------------------------------------------------------|-----------------------------------------------------|---|---|
| 1       | —H             | 5'-Cl                                                                               | II             | 5'-Cl                            | C <sub>2</sub> H <sub>5</sub> | (CH <sub>2</sub> ) <sub>3</sub> SO <sub>3</sub> <sup>-</sup> | (CH <sub>2</sub> ) <sub>3</sub> SO <sub>3</sub> H   | — | 1 |
| 2       | —H             | 5-COOCH <sub>3</sub>                                                                | II             | 5'-COOCH <sub>3</sub>            | C <sub>2</sub> H <sub>5</sub> | (CH <sub>2</sub> ) <sub>3</sub> SO <sub>3</sub> <sup>-</sup> | (CH <sub>2</sub> ) <sub>3</sub> SO <sub>3</sub> H   | — | 1 |
| 3       | —H             | 5-F                                                                                 | II             | 5'F                              | C <sub>2</sub> H <sub>5</sub> | (CH <sub>2</sub> ) <sub>3</sub> SO <sub>3</sub> <sup>-</sup> | (CH <sub>2</sub> ) <sub>3</sub> SO <sub>3</sub> H   | — | 1 |
| 4       | —H             | 5-Br                                                                                | II             | 5'-Br                            | C <sub>2</sub> H <sub>5</sub> | (CH <sub>2</sub> ) <sub>3</sub> SO <sub>3</sub> <sup>-</sup> | (CH <sub>2</sub> ) <sub>3</sub> SO <sub>3</sub> H   | — | 1 |
| 5       | —H             | 5-OCH <sub>3</sub>                                                                  | II             | 5'-OCH <sub>3</sub>              | C <sub>2</sub> H <sub>5</sub> | (CH <sub>2</sub> ) <sub>3</sub> SO <sub>3</sub> <sup>-</sup> | (CH <sub>2</sub> ) <sub>3</sub> SO <sub>3</sub> H   | — | 1 |
| 6       | —H             | 5-CH <sub>3</sub>                                                                   | II             | 5'-CH <sub>3</sub>               | C <sub>2</sub> H <sub>5</sub> | (CH <sub>2</sub> ) <sub>3</sub> SO <sub>3</sub> <sup>-</sup> | (CH <sub>2</sub> ) <sub>3</sub> SO <sub>3</sub> H   | — | 1 |
| 7       | —II            |  | II             | 5'-C <sub>2</sub> H <sub>5</sub> | C <sub>2</sub> H <sub>5</sub> | (CH <sub>2</sub> ) <sub>3</sub> SO <sub>3</sub> <sup>-</sup> | (CH <sub>2</sub> ) <sub>3</sub> SO <sub>3</sub> HII | — | 1 |

(The numbers on the left side in the columns A<sub>2</sub> and A<sub>4</sub> represent the position of the substituent.)

TABLE 2

Examples of dyes belonging to those represented by the general formula (2) are:

TABLE 2—Continued

| Dye No. | B <sub>1</sub> | B <sub>2</sub> | B <sub>3</sub>     | B <sub>4</sub> | R <sub>3</sub>                | R <sub>4</sub>                                               | R <sub>5</sub>                | R <sub>6</sub> | Y                                | X    | m |
|---------|----------------|----------------|--------------------|----------------|-------------------------------|--------------------------------------------------------------|-------------------------------|----------------|----------------------------------|------|---|
| 15      | 6-Cl           | 5-Cl           | 6'-Cl              | 5'-Cl          | C <sub>2</sub> H <sub>5</sub> | C <sub>2</sub> H <sub>5</sub>                                | C <sub>2</sub> H <sub>5</sub> | H              | >N—C <sub>2</sub> H <sub>5</sub> | SCN— | 2 |
| 16      | 6-Cl           | 5-Cl           | 5'-CH <sub>3</sub> | 6'-H           | C <sub>2</sub> H <sub>5</sub> | (CH <sub>2</sub> ) <sub>3</sub> SO <sub>3</sub> <sup>—</sup> | CH <sub>3</sub>               | II             | CH <sub>3</sub>                  |      | 1 |



The numeral on the left side in the columns B<sub>1</sub>, B<sub>2</sub>, B<sub>3</sub> and B<sub>4</sub> represents the position of the substituent.

As is described above, iodide ions and the green sensitizing dyes are added to a sol-state photographic emulsion to adsorb them onto the surface of the silver bromoiodide grains contained therein. The molar ratio of a water-soluble iodide to a green sensitizing dye added is preferred to be within a range of from more than 1 to about 6. The green sensitizing dye employed is preferably a dye without an iodide counter anion when the ratio is near 1. After further adding to this emulsion other known additives for photographic emulsions (such as stabilizers, hardeners, coating aids, and the like), the sol-state photographic emulsion is applied to a support film comprising cellulose triacetate, polyethylene terephthalate, etc., at a uniform thickness, set with cold air and then dried by blowing a large amount of air with low moisture and at high temperature over the film. Thus, there can be obtained the desired photographic light-sensitive material.

#### EXAMPLE 1

A negative-working photographic emulsion comprising silver bromoiodide grains having a mean grain diameter of 0.7  $\mu$  and containing 7.1 mol percent of io-

10 Davis-Gibson filter) under an illuminance of 100 lux at the exposure surface for 1/100 second through a yellow filter and a neutral continuous wedge, the yellow filter cutting blue light and thus enabling one to measure only the sensitivity of the spectrally sensitized region.

15 The exposed samples were developed in the following developer at 20°C for 6 minutes.

#### Developer Composition:

|    |                                                                                        |           |
|----|----------------------------------------------------------------------------------------|-----------|
| 20 | Monol (Trade name used by Fuji Photo Film Co., Ltd for N-methyl-p-aminophenyl sulfate) | 4.5 g     |
|    | Sodium sulfite (anhydrous)                                                             | 50 g      |
|    | Hydroquinone                                                                           | 4.5 g     |
|    | Sodium carbonate (monohydrate)                                                         | 35 g, and |
|    | Potassium bromide                                                                      | 2 g       |

25 Added successively to 1 liter of water.

Immediately after the development, the materials were processed in a stopping bath (0.3 percent glacial acetic acid soln.), then in a fixing bath (Kodak F-5 solution; "Kodak" is a registered trade mark), washed and dried. The optical density of the silver image formed was measured, and the sensitivity was determined from the reciprocal of the exposure required to obtain an optical density of 0.5 above fog. The results obtained are shown in Table 4.

Table 4

| Sample No.                 | I    | II  | III | IV  | V   | VI  | VII | VIII |
|----------------------------|------|-----|-----|-----|-----|-----|-----|------|
| Sensitivity                | 100* | 145 | 160 | 160 | 200 | 225 | 200 | 320  |
| Peak wavelength (m $\mu$ ) | 550  | 550 | 550 | 550 | 550 | 550 | 565 | 565  |

\* Taken as 100 as a standard for comparison convenience.

dide ion (based on the amount of silver ion) and gelatin (grains/gelatin = 1.18 wt. ratio) was kept in a sol-state at 35°C. To this emulsion were added the solutions of potassium iodide and the green sensitizing dye(s) each in an amount as is given in Table 3 to adsorb the same on said grains.

45 The addition of potassium iodide in an amount of more than 100 mg did not further increase the sensitivity. On the contrary, development was delayed by such addition.

As can be seen in the above Table, in the region wherein a significant increase in sensitivity cannot be ex-

Table 3

| Sample No.<br>Additives | I     | II    | III   | IV    | V     | VI    | VII   | VIII  |
|-------------------------|-------|-------|-------|-------|-------|-------|-------|-------|
| Potassium iodide*       | —     | —     | —     | 20mg  | 50mg  | 100mg | —     | 50mg  |
| Dye No. 1**             | 130mg | 200mg | 270mg | 200mg | 200mg | 200mg | 200mg | 200mg |
| Dye No. 13**            | —     | —     | —     | —     | —     | 50mg  | 50mg  | 50mg  |

(All of the amounts added are per 1 mol of silver)

\*Added as a 0.1% aqueous solution.

\*\*Added as a 0.1% methanol solution.

The resulting emulsions (sol state) were applied on to a cellulose triacetate film base in a coating amount of 15 mg of silver/dm<sup>2</sup> to a thickness of 5  $\mu$  (after drying), and then dried.

The materials thus obtained were exposed to light of 4,800°K (a tungsten lamp provided with a prescribed

65 pected by increasing the amount of the dye (1) added, a further increase in sensitivity can be obtained by using potassium iodide together with the dye(s). In addition, in this case, the suitable amount lies between 50 and 100 mg of potassium iodide per mol of silver.

It can also be seen that for the combination of dye

(1) and dye (13), potassium iodide is similarly effective for sensitization. This combination gives green sensitivity of an approximately 15 m $\mu$  longer peak wavelength than that obtained by the use of dye 1, but the speed is kept equal between the two by the addition of an appropriate amount of iodide according to the invention, as seen from the comparison of sample V and VII in Table 3 and 4 above. Such a dye combination is another embodiment of the present invention.

**EXAMPLE 2**

Dyes given in Table 5 were added to the same silver bromoiodide photographic emulsion as in Example 1. In this example, the amount of potassium iodide added was fixed. The sensitivity of each of these samples was measured in the same manner as in Example 1 to obtain the results given in Table 5.

(after drying) of  $5 \mu$  to the same support as in Example 1 which had been coated with an antihalation layer comprising  $1.4 \text{ mg/dm}^2$  of colloidal silver particles dispersed in  $2.14 \text{ g/m}^2$  of gelatin and a red sensitive layer (containing  $0.8 \text{ g/m}^2$  of N-n-dodecyl-1-hydroxy-2-naphthoic acid amide as a cyan coupler,  $1.2 \text{ g/m}^2$  of silver as silver iodobromide grains and red sensitizing dye as the major constituents of this layer).

Onto the resulting green sensitive layer were applied 10 successively a colloidal silver yellow filter layer, a blue sensitive layer (containing 4-dodecyl-benzoyl-2-methoxy-acetanilide yellow coupler), and a protective film layer to obtain a color light-sensitive material.

The sensitivity of the light-sensitive material thus obtained was measured in the same manner as in Example 1 except for the following procedure: the yellow filter was not employed in the exposure and therefore the

Table 5

| Sample No.                          | IX           | X            | XI           | XII          | XIII         | XIV          | XV           | XVI          | XVII         | XVIII        |
|-------------------------------------|--------------|--------------|--------------|--------------|--------------|--------------|--------------|--------------|--------------|--------------|
| Added dye No.<br>and the amount     | (2)<br>200mg | (2)<br>200mg | (3)<br>200mg | (3)<br>200mg | (4)<br>200mg | (4)<br>200mg | (5)<br>200mg | (5)<br>200mg | (6)<br>200mg | (6)<br>200mg |
| Amount of potassium<br>iodide added | —            | 85mg         | —            | 85mg         | —            | 85mg         | —            | 85mg         | —            | 85mg         |
| Sensitivity*                        | 35           | 45           | 50           | 100          | 35           | 40           | 35           | 140          | 12           | 32           |
| Peak wavelength<br>( $\mu$ )        | 540          | 540          | 525          | 525          | 550          | 550          | 545          | 545          | 535          | 535          |

(Amounts added are per 1 mol of silver)

\* The sensitivity of sample No. 1 is taken as 100.

### EXAMPLE 3

An example of applying the photographic emulsion of the invention to a green sensitive layer of a color lightsensitive material is shown below.

The same silver bromoiodide gelatin emulsions as in Example 1 were maintained at 35°C in a sol state, and potassium iodide and the green sensitizing dye(s) were added thereto as a 0.1 percent aqueous solution and a 0.1 percent methanol solution, respectively, each in an amount as given in Table 6. Thereafter, the resulting emulsions were left for 30 minutes while stirring so as to adsorb the iodide and dye(s) sufficiently on the surface of the grains. Then, the following additives (per 1 mol of silver) were added thereto successively: 60 ml of a 0.5 percent aqueous solution of 5-methyl-7-hydroxy-1,3,4-triazaindolizine as a stabilizer; 70 g of 1-(2,4,6-trichloro)-phenyl-3-dodecylamido-5-pyrazolone (as a magenta coupler) dissolved in mixture of 70 g of tricresyl phosphate and 100 ml of ethyl acetate under heating and subsequently dispersed in 700 g of a 10 weight percent gelatin aqueous solution in the presence of 84 ml of a 5 percent sodium dodecylsulfate aqueous solution; 20 ml of a 2 percent aqueous solution of 2,6-dichloro-4-hydroxy-triazine; and 3 ml of a 4 percent aqueous solution of saponin.

The resulting photographic emulsion was applied to provide an amount of silver of  $18 \text{ mg}/\text{dm}^2$  to a thickness

light-sensitive material was directly exposed to the light source of 4,800°K. To the developer there was further added 1.5 g (per liter) of potassium thiocyanate, and development was conducted at 24°C for 10 minutes. After development, the light-sensitive material was processed in a stopping bath and subsequently exposed to a strong diffuse white light over the entire surface to fog the material. Thereafter, color development was conducted at 24°C for 15 minutes in the following color developer to obtain a color positive image.

### Composition of the Color Developer:

|                                                                                 |            |
|---------------------------------------------------------------------------------|------------|
| Benzyl alcohol                                                                  | 5.0 ml     |
| Sodium sulfite (anhydrous)                                                      | 5.0 g      |
| Trisodium phosphate (12 hydrate)                                                | 40 g       |
| Sodium hydroxide                                                                | 1.5 g      |
| Potassium bromide                                                               | 0.5 g      |
| Ethylenediamine                                                                 | 5.0 ml     |
| Citrazinic acid                                                                 | 1.5 g, and |
| p-Amino-N-ethyl-N- $\beta$ -methanesulfone-<br>amidoethyl-m-toluidine sulfonate | 10.5 g     |

were added successively per 1 liter of water.

Subsequently, washing, bleaching, fixing and washing were conducted to obtain a color image. The optical density of the magenta image therein were measured through a green filter, which was represented by the reciprocal of the exposure providing a density of 0.5. The results obtained are given in the following Table.

Table 6

Table 6—Continued

| Sample No.                       | XIX  | XX  | XXI         | XXII        | XXIII | XXIV | XXV         | XXVI        | XXVII | XXVIII | XXIX | XXX | XXXI | XXXII |
|----------------------------------|------|-----|-------------|-------------|-------|------|-------------|-------------|-------|--------|------|-----|------|-------|
| amount of potassium iodide added |      |     |             |             |       |      |             |             |       |        |      |     |      |       |
| Sensitivity                      | 100* | 150 | 135         | 240         | 55    | 64   | 55          | 65          | 40    | 70     | 45   | 55  | 80   | 95    |
| Peak wavelength (m $\mu$ )       | 565  | 565 | 540+<br>565 | 540+<br>565 | 565   | 565  | 535+<br>570 | 535+<br>570 | 560   | 560    | 555  | 555 | 560  | 560   |

(per 1 mol of silver)

\* 100 taken as the standard.

From Table 6 above, the excellent effect of the present invention can be understood to be provided similarly to the case of Example 2.

## EXAMPLE 4

The same silver bromoiodide photographic emulsion as in Example 1 was maintained in a sol state at 35°C, and an aqueous solution of potassium iodide and a methanol solution of dye(s) were added thereto as shown in Table 7 to adsorb the dye(s) and iodide onto the grains. The resulting emulsions were applied and dried in the same manner as in Example 1, and subsequently subjected to sensitometry measurements to thereby obtain the sensitivity data shown in the following Table. In the case of using these dyes too, the same effect of potassium iodide as was illustrated in the foregoing Examples can clearly be recognized.

Table 7

| Sample No.                       | XXXIII | XXXIV | XXXV  | XXXVI       | XXXVII      |
|----------------------------------|--------|-------|-------|-------------|-------------|
| Amount of potassium iodide added | —      | —     | 85mg  | —           | 85mg        |
| Amount of dye added (16)         | —      | 200mg | 200mg | 200mg       | 200mg       |
| Amount of dye added (13)         | 50mg   | —     | —     | 50mg        | 50mg        |
| Amount of dye added (1)          | 200mg  | —     | —     | —           | —           |
| Sensitivity measurements         | 100 *  | 25    | 40    | 55          | 90          |
| Peak wavelength (m $\mu$ )       | 565    | 535   | 535   | 535+<br>565 | 535+<br>565 |

(Amounts added were per 1 mol of silver)

\* 100 taken as the standard.

While the invention has been described in detail and with reference to specific embodiments thereof, it will be apparent to one skilled in the art that various changes and modifications can be made therein without departing from the spirit and scope thereof.

What is claimed is:

1. In a silver bromoiodide negative-working photographic emulsion of the developing out type which is subjected to only one exposure followed by wet-developing, said emulsion containing at least one green sensitizing dye to effect green sensitization thereof, a silver bromoiodide photographic emulsion wherein at least 0.01 mol percent of iodide ion based on silver halide adsorbs on the surface of silver bromoiodide grains contained in the emulsion, said iodide ion being in ad-

dition to iodine present in said silver iodobromide grains and said green sensitizing dye intensely sensitizing said emulsion to green without substantially deteriorating its photographic properties wherein said green sensitizing dye is represented by one of the following general formulae



wherein  $A_1$  and  $A_3$  each represents a hydrogen atom or halogen atom,  $A_2$  and  $A_4$  represent a hydrogen atom, halogen atom, hydroxy group, alkoxy group, amino group, acylamido group, acyloxy group, alkoxy carbonyl group, lower alkyl group or alkoxy carbonyl group, or, when taken together,  $A_1$  and  $A_2$ , and  $A_3$  and  $A_4$ , can be the atoms necessary to form a benzene nucleus, R represents a hydrogen atom, lower alkyl group, or aryl group,  $R_1$  and  $R_2$  each represents an alkyl group, hydroxyalkyl group, acetoxyalkyl group, alkoxyalkyl group, alkyl group containing a carboxyl group, alkyl group containing sulfo group, benzyl group, phenethyl group or a vinylmethyl group; and



wherein  $B_1$  represents a hydrogen atom or halogen atom,  $B_2$ ,  $B_3$  and  $B_4$  each represents a hydrogen atom, halogen atom, lower alkyl group, amino group, acylamido group, acyloxy group, alkoxy carbonyl group, carboxyl group, alkoxy group, aryl group, cyano group, carbamoyl group, alkylsulfonyl group, alkylaminosulfonyl group or aminosulfonyl group, or, when taken together,  $B_3$  and  $B_4$ , can represent the atoms necessary to form a benzene ring, Y represents  $-O-$

13



wherein R<sub>7</sub> and R<sub>8</sub> each represents an alkyl group,



wherein R<sub>9</sub> represents an alkyl group, R<sub>3</sub>, R<sub>4</sub> and R<sub>5</sub> represent the same alkyl groups as R<sub>1</sub> or R<sub>2</sub>; R<sub>6</sub> represents a hydrogen atom or R<sub>5</sub> and R<sub>6</sub> may combine with each other through an alkylene group, and m represents 1 or 2.

2. The photographic emulsion as claimed in claim 1, wherein bromide ion in an amount of from 1 to 30 times of the molar concentration of the iodide ion added is also adsorbed on the surface of silver bromoiodide grains contained in the emulsion.

3. The photographic emulsion as claimed in claim 1 comprising silver bromoiodide mixed crystals with about 0.01 to about 1.0 mol percent of iodide ions adsorbed on the surface thereof.

4. The photographic emulsion as claimed in claim 1, wherein the green sensitizing dye is an anionic dye.

5. The photographic emulsion as claimed in claim 1, wherein the green sensitizing dye is a cationic dye without an iodide ion as a counter anion.

6. The photographic emulsion as claimed in claim 1, wherein the amount of said iodide ions added is at least 0.05 mol percent based on silver halide and the green sensitizing dye is a cationic dye with an iodide ion as a counter anion.

7. The photographic emulsion as claimed in claim 1, wherein the amount of said iodide ions added is within the range of from 0.05 to 0.3 mol percent based on silver halide.

8. The photographic emulsion as claimed in claim 1, wherein at least two of said dyes are used in combination.

9. The photographic emulsion as claimed in claim 1, wherein the halogen atom in A<sub>1</sub>, A<sub>3</sub> or B<sub>1</sub> is chlorine, bromine, iodine or fluorine; wherein the alkoxy group is methoxy or ethoxy, the amino group is amino, methylamino or dimethylamino, the acylamido group is acetoamido or propionamido, the acyloxy group is acetoxy, the alkoxy carbonyl group is methoxycarbonyl, ethoxycarbonyl, propioxy carbonyl or butoxy carbonyl in A<sub>2</sub>, A<sub>4</sub>, B<sub>2</sub>, B<sub>3</sub> or B<sub>4</sub>; the lower alkyl group is methyl, ethyl or isopropyl in A<sub>2</sub> or A<sub>4</sub>; wherein the lower alkyl group is methyl, ethyl or n-propyl, and the aryl group is phenyl or tolyl in R<sub>4</sub>; wherein the alkyl group is methyl, ethyl or n-propyl, the hydroxyalkyl group is 2-hydroxyethyl, 3-hydroxypropyl or 4-hydroxybutyl, the acetoxyalkyl group is 2-acetoxyethyl, 3-acetoxypropyl or 4-acetoxybutyl, the alkoxyalkyl group is 2-methoxyethyl or 3-methoxypropyl, the alkyl group containing a carboxy group is carboxymethyl, 2-carboxyethyl, 3-carboxypropyl, 4-carboxybutyl or 2-(2-carboxyethoxy)ethyl, the alkyl group containing a sulfo group is 2-sulfoethyl, 3-sulfopropyl, 4-sulfobutyl, 2-hydroxy-3-sulfopropyl, 2-(3-sulfopropoxy)ethyl, 2-acetoxy-3-sulfopropyl, 3-methoxy-2-(3-sulfopropoxy)propyl, 2-[2-(3-sulfopropoxy)ethoxy]ethyl, p-sulfobenzyl, p-sulfobenzyl or p-sulfophenethyl in R<sub>1</sub>, R<sub>2</sub>, R<sub>3</sub>, R<sub>4</sub> or R<sub>5</sub>; wherein the lower alkyl group is methyl, ethyl or trifluoromethyl, the aryl group is phe-

14

nyl or tolyl, the carbamoyl group is carbamoyl, methylcarbamoyl, phenylcarbamoyl, dimethylcarbamoyl, diethylcarbamoyl, morpholinocarbamoyl or piperidino-carbamoyl, the alkyl sulfonyl group is methyl sulfonyl, the alkylaminosulfonyl group is methylaminosulfonyl, ethylaminosulfonyl, dimethylaminosulfonyl, morpholinosulfonyl, piperidinosulfonyl or pyrrolidinosulfonyl in B<sub>2</sub>, B<sub>3</sub> or B<sub>4</sub>; wherein the alkyl group in R<sub>7</sub> or R<sub>8</sub> is methyl, ethyl or vinylmethyl; wherein the alkyl group is R<sub>9</sub> is methyl or ethyl; and wherein the alkylene group, which joins together R<sub>5</sub> and R<sub>6</sub>, is dimethylene or trimethylene.

10. The photographic emulsion as claimed in claim 1, wherein said green sensitizing dye is a cyanine dye selected from the group:



11. The photographic emulsion as claimed in claim 1, wherein more than one green sensitizing dye is used, the dyes comprising a combination of:



12. The photographic emulsion as claimed in claim 1, wherein the amount of green sensitizing dye is within the range of from 10<sup>-4</sup> to 2 × 10<sup>-2</sup> moles per 1 mole of silver halide.

13. The photographic emulsion as claimed in claim 1, wherein the emulsion comprises a hydrophilic colloid selected from the group gelatin, phthalated gelatin, polyacrylic amide, polyvinyl alcohol and polyvinyl pyrrolidone.

14. The photographic emulsion as claimed in claim 1, further containing a coupler.

15. The photographic light-sensitive silver halide material which comprises a support having thereon at least one layer comprising a photographic emulsion as claimed in claim 1.

16. In a process for spectrally sensitizing a negative-working silver bromoiodide photographic emulsion of the developing out type which is subjected to only one exposure followed by wet-developing, said emulsion containing at least one green sensitizing dye which effects the green sensitization of said emulsion, the improvement comprising adsorbing at least 0.1 mol percent iodide ions on the surface of the silver halide grains in the emulsion, said iodide being in addition to iodine present in said silver iodobromide, whereby the emulsion is intensely sensitized to green without substantially deteriorating its photographic properties wherein said green sensitizing dye is represented by one of the following general formulae



wherein A<sub>1</sub> and A<sub>3</sub> each represents a hydrogen atom or halogen atom, A<sub>2</sub> and A<sub>4</sub> represent a hydrogen atom, halogen atom, hydroxy group, alkoxy group, amino group, acylamido group, acyloxy group, aloxycarbonyl group, lower alkyl group or aloxycarbonylamino group, or, when taken together, A<sub>1</sub> and A<sub>2</sub>, and A<sub>3</sub> and A<sub>4</sub>, can be the atoms necessary to form a benzene nucleus, R represents a hydrogen atom, lower alkyl group, or aryl group, R<sub>1</sub> and R<sub>2</sub> each represents an alkyl group, hydroxyalkyl group, acetoxyalkyl group, alkoxyalkyl group, alkyl group containing a carboxyl group, alkyl group containing sulfo group, benzyl group, phenethyl group or a vinylmethyl group; and



wherein B<sub>1</sub> represents a hydrogen atom or halogen atom, B<sub>2</sub>, B<sub>3</sub> and B<sub>4</sub> each represents a hydrogen atom, halogen atom, lower alkyl group, amino group, acylamino group, acyloxy group, aloxycarbonyl group, carboxyl group, alkoxy group, aryl group, cyano group, carbamoyl group, alkylsulfonyl group, alkylaminosulfonyl group or aminosulfonyl group, or, when taken together, B<sub>3</sub> and B<sub>4</sub>, can represent the atoms necessary to form a benzene ring, Y represents —O—



wherein R<sub>7</sub> and R<sub>8</sub> each represents an alkyl group.



5

wherein R<sub>9</sub> represents an alkyl group, R<sub>3</sub>, R<sub>4</sub> and R<sub>5</sub> represent the same alkyl groups as R<sub>1</sub> or R<sub>2</sub>; R<sub>6</sub> represents a hydrogen atom or R<sub>5</sub> and R<sub>6</sub> may combine with each other through an alkylene group, and m represents 1 or 2.

17. The process as claimed in claim 16, wherein bromide ion in an amount of from 1 to 30 times of the molar concentration of the iodide ion added is also adsorbed on the surface of silver bromoiodide grains contained in the emulsion.

18. The process as claimed in claim 16, wherein said emulsion comprises silver bromoiodide mixed crystals with about 0.01 to about 1.0 mol percent of iodide ions adsorbed on the surface thereof.

19. The process as claimed in claim 16, wherein the amount of said iodide ions added is within the range of from 0.05 to 0.3 mol percent based on silver halide.

20. The process as claimed in claim 16, wherein at least two of said dyes are used in combination.

21. The process as claimed in claim 16, wherein the halogen atom in A<sub>1</sub>, A<sub>3</sub> or B<sub>1</sub> is chlorine, bromine, iodine or fluorine; wherein the alkoxy group is methoxy or ethoxy, the amino group is amino, methylamino or

30 dimethylamino, the acylamido group is acetoamido or propionamido; the acyloxy group is acetoxy, the alkoxycarbonyl group is methoxycarbonyl, ethoxycarbonyl, propioxycarbonyl or butoxycarbonyl in A<sub>2</sub>, A<sub>4</sub>, B<sub>2</sub>, B<sub>3</sub> or B<sub>4</sub>; the lower alkyl group is methyl, ethyl or isopropyl in A<sub>2</sub> or A<sub>4</sub>; wherein the lower alkyl group is methyl, ethyl or n-propyl, and the aryl group is phenyl or tolyl in R<sub>4</sub> wherein the alkyl group is methyl, ethyl or n-propyl, the hydroxyalkyl group is 2-hydroxyethyl, 3-hydroxypropyl or 4-hydroxybutyl, the acetoxyalkyl group is 2-acetoxyethyl, 3-acetoxypropyl or 4-acetoxybutyl, the alkoxyalkyl group is 2-methoxyethyl or 3-methoxypropyl, the alkyl group containing a carboxy group is carboxymethyl, 2-carboxyethyl, 3-carboxypropyl, 4-carboxybutyl or 2-(2-carboxyethoxy)ethyl, the alkyl group containing a sulfo group is 2-sulfoethyl, 3-sulfopropyl, 4-sulfobutyl, 2-hydroxy-3-sulfopropyl, 2-(3-sulfopropoxy)ethyl, 2-acetoxy-3-sulfopropyl, 3-methoxy-2-(3-sulfopropoxy)propyl, 2-[2-(3-sulfopropoxy)-ethoxy]ethyl, p-sulfobenzyl, p-sulfobenzyl or p-sulfophenethyl in R<sub>1</sub>, R<sub>2</sub>, R<sub>3</sub>, R<sub>4</sub> or R<sub>5</sub>; wherein the lower alkyl group is methyl, ethyl or trifluoromethyl, the aryl group is phenyl or tolyl, the carbamoyl group is carbamoyl, methylcarbamoyl, phenylcarbamoyl, dimethylcarbamoyl, diethylcarbamoyl

40 morpholinocarbamoyl or piperidinocarbamoyl, the alkyl sulfonyl group is methyl sulfonyl, the alkylaminosulfonyl group is methylaminosulfonyl, ethylaminosulfonyl, dimethylaminosulfonyl, morpholinosulfonyl, piperidinosulfonyl or pyrrolidinosulfonyl in B<sub>2</sub>, B<sub>3</sub> or B<sub>4</sub>; wherein the alkyl group in R<sub>7</sub> or R<sub>8</sub> is methyl, ethyl or vinylmethyl; wherein the alkyl group in R<sub>9</sub> is methyl or ethyl; and wherein the alkylene group, which joins together R<sub>5</sub> and R<sub>6</sub>, is dimethylene or trimethylene.

55 22. The process as claimed in claim 16, wherein said green sensitizing dye is a cyanine dye selected from the group:

17



and



23. The process as claimed in claim 16, wherein more than one green sensitizing dye is used, the dyes comprising a combination of:



and



18

or



10 24. The process as claimed in claim 16, wherein the amount of green sensitizing dye is within the range of from  $10^{-4}$  to  $2 \times 10^{-2}$  moles per 1 mole of silver halide.

15 25. The photographic emulsion of claim 1 which has been chemically ripened.

16 26. The process of claim 16, wherein said photographic emulsion has been chemically ripened.

17 27. The photographic emulsion of claim 1, wherein more than 1 green sensitizing dye is used, the spectral absorption regions of the green sensitizing dyes differing from each other.

18 28. The process of claim 16, wherein more than 1 green sensitizing dye is used, the spectral absorption regions of the green sensitizing dyes differing from each other.

19 29. The photographic emulsion as claimed in claim 1 wherein said silver bromoiodide mixed crystals contain about 0.5 to about 10 mol percent of iodide ions based on the total silver halide.

20 30. The process as claimed in claim 16, wherein said silver bromoiodide mixed crystals used contain about 0.05 to about 10 mol percent of iodide ions based on the total silver halide.

21 31. The photographic emulsion as claimed in claim 1 wherein the green sensitizing dye is cationic.

22 32. The process as claimed in claim 16, wherein the green sensitizing dye is cationic.

40

\* \* \* \* \*

45

50

55

60

65